

## UNITED STATES PATENT OFFICE

2,550,449

ELECTRODEPOSITION OF NICKEL FROM  
AN ACID BATHHenry Brown, Detroit, Mich., assignor to The  
Udylite Corporation, Detroit, Mich., a corpora-  
tion of DelawareNo Drawing. Application April 20, 1946,  
Serial No. 663,757

2 Claims. (Cl. 204—49)

1

This invention relates to the electrodeposition of bright ductile plate from aqueous acidic nickel baths.

This object can be accomplished by the addition of certain soluble unsaturated organic compounds selected from the class of N-alkyl pyridinium and quinolinium pyrazoles (such, e. g., as the compounds listed in Table I) to acidic nickel baths (such, e. g., as those listed in Table II), and containing in addition vinyl sulfonic or allyl sulfonic acid or one or more of the alpha or beta unsaturated aliphatic sulfonic acids or sulfonates listed in Table III.

While the alpha or beta unsaturated aliphatic sulfonic acids such as those listed in Table III (see application Serial No. 603,753, now Patent No. 2,523,190) produce bright plate on buffed surfaces, the rate of brightening of a dull surface is rather slow, that is, they do not improve the brightness of the original surface at a very rapid rate. If, however, one or more of the active unsaturated compounds listed in Table I is added to the acidic nickel bath containing, for example, vinyl or allyl sulfonate, then the brightness and the rate of brightening is greatly improved.

The compounds of Table III have no upper limit in concentration except their solubility in the bath. After the optimum concentration is reached (usually from 1-5 g./l.), further additions produce little further improvement. Concentrations as low as 0.1 g./l. make noticeable improvement of the lower current density areas. With respect to their ability of keeping the lowest current density areas bright and adherent despite the presence of appreciable amounts of zinc, the vinyl and allyl sulfonic acids are quite remarkable.

The compounds of Table I are preferably used at their optimum concentrations, though higher concentrations can be used, for example, if the bath is used at the lower temperatures such as room temperature. In general, the higher the temperature, and the greater the degree of agitation at the cathode surface, the smaller the concentration of the compounds of Table I for optimum results. To obtain a desirable bright plate, one or more of the compounds of Table I preferably is used in an amount falling within a range from about .001 gram per liter to about .02 gram per liter of solution with one or more of the compounds of Table III, but excessively high concentrations will produce brittleness.

The compounds of Table I should not be used

in concentrations above about .02 g./l. or else the plate will be made brittle. Also, it is preferred that the N-alkyl chain be less than about 8 carbon atoms or it will confer upon the compounds the properties of cationic wetting agents which will then cancel out or agglomerate with any anionic wetting agents that may be present for the prevention of pitting. In particular the N-methyl chloracetate or N-ethyl chloracetate (or the betaine form) are desirable (Nos. 11, 12) as they are the least critical to obtain the highest brightness without serious embrittlement or darkening of the lowest current density areas. Compounds Nos. 1, 2, 6, 11 and 12 are the best members to use of Table I, from the standpoint of excellent effectiveness and least difficulty of preparation.

The compounds of Table III are remarkable in their making possible the use of higher concentrations of the compounds of Table I in the baths without seriously impairing the ductility, besides making very bright plate possible. Even the very lowest current density areas are made bright by the use of compounds of Table III.

TABLE I

| Compound No. |                                                                             | Opt. Cone. in Bath, g./l. |
|--------------|-----------------------------------------------------------------------------|---------------------------|
| 1            | N-ethanol (β-hydroxy ethyl), 4-nitro-5-(3'-pyridinium) pyrazole chloride    | 0.002-0.08                |
| 2            | N-ethanol, 3-nitro-5-(3' pyridinium) pyrazole chloride                      | 0.002-0.08                |
| 3            | N-ethanol, 3,4-di-nitro-5-(3' pyridinium) pyrazole chloride                 | 0.002-0.08                |
| 4            | N-β,α, dihydroxy propyl-4-nitro-5-(3'-pyridinium) pyrazole chloride         | 0.002-0.08                |
| 5            | N-acetyl-4-nitro-5-(3' pyridinium) pyrazole chloride                        | 0.002-0.08                |
| 6            | N-allyl-4-nitro-5-(3'-pyridinium) pyrazole bromide                          | 0.002-0.08                |
| 7            | N-butanol-4-nitro-5-(3'-pyridinium) pyrazole iodide                         | 0.002-0.08                |
| 8            | N-ethyl-5-(3'-pyridinium) pyrazole sulfate                                  | 0.002-0.08                |
| 9            | N-ethanol-5-(3'-isoquinolinium) pyrazole chloride                           | 0.002-0.08                |
| 10           | N-ethanol-1-(2'-quinolinium) pyrazole chloride                              | 0.002-0.08                |
| 11           | N-methyl or ethyl acetate-4-nitro-5-(3'-pyridinium) pyrazole chloride       | 0.002-0.08                |
| 12           | N-acetic acid (or betaine form)-4-nitro-5-(3'-pyridinium) pyrazole chloride | 0.002-0.08                |



sulfonimides (such, e. g., as the allyl or vinyl sulfonamides or sulfonimides) may be used. These compounds show beneficial effects in concentrations as low as .1 g./l. and can be used effectively in concentrations as high as saturation in the bath.

I claim:

1. A bath for electrodepositing bright nickel consisting essentially of an aqueous acid solution of a material selected from the group consisting of nickel chloride, nickel sulfate, a mixture of nickel sulfate and nickel chloride, a mixture of nickel fluoborate and nickel chloride, a mixture of nickel fluoborate and nickel sulfate, and a mixture of nickel sulfate, nickel chloride, and nickel fluoborate, said solution also containing in a concentration falling within a range of from about .1 gram per liter to saturation an organic compound soluble in the solution and selected from the group consisting of allyl sulfonic acids, allyl and vinyl sulfonamides and sulfonimides, said solution also containing in a concentration falling within a range of from about .001 gram per liter to .02 gram per liter a compound selected from the group consisting of N-aliphatic pyridinium pyrazoles and N-aliphatic quinolinium pyrazoles, the N-aliphatic group containing from 1 to 8 carbon atoms, said bath having a pH of from about 1 to 6.

2. The method of electrodepositing bright nickel comprising the step of electrodepositing bright nickel from an aqueous acid solution of a material selected from the group consisting essentially of nickel chloride, nickel sulfate, a mixture of nickel sulfate and nickel chloride, a mixture of nickel fluoborate and nickel chloride, a mixture of nickel fluoborate and nickel sulfate, and a mixture of nickel sulfate, nickel chloride, and nickel fluoborate, said solution also contain-

ing in a concentration falling within a range of from about .1 gram per liter to saturation an organic compound soluble in the solution and selected from the group consisting of allyl sulfonic acids, allyl and vinyl sulfonamides and sulfonimides, said solution also containing in a concentration falling within a range of from about .001 gram per liter to .02 gram per liter a compound selected from the group consisting of 10 N-aliphatic pyridinium pyrazoles and N-aliphatic quinolinium pyrazoles, the N-aliphatic group containing from 1 to 8 carbon atoms, said bath having a pH of from about 1 to 6.

HENRY BROWN.

15

#### REFERENCES CITED

The following references are of record in the file of this patent:

| UNITED STATES PATENTS |           |             |                |
|-----------------------|-----------|-------------|----------------|
|                       | Number    | Name        | Date           |
| 20                    | 2,029,387 | Pine        | Feb. 4, 1936   |
|                       | 2,191,813 | Brown       | Feb. 27, 1940  |
|                       | 2,198,267 | Lind et al. | Apr. 23, 1940  |
| 25                    | 2,255,057 | Holt        | Sept. 9, 1941  |
|                       | 2,315,802 | Lind et al. | Apr. 6, 1943   |
|                       | 2,427,280 | Hoffman     | Sept. 9, 1947  |
|                       | 2,513,280 | Brown       | July 4, 1950   |
| 30                    | 2,523,190 | Brown       | Sept. 19, 1950 |
|                       | 2,523,191 | Brown       | Sept. 19, 1950 |

#### OTHER REFERENCES

- Metal Industry, Nov. 24, 1944, p. 331.  
 Modern Electroplating, published by Electrochemical Society (1942), pp. 242, 243.  
 35 Davis et al.: Ind. and Eng. Chem., vol. 33, pp. 1546 and 1547 (1941).  
 Organic Chemistry by Frank C. Whitmore, 1937, D. Van Nostrand Co., N. Y., pp. 902, 941, 943, 40 944, 948, 951, 952.